

3,420,661

## ZINC BASE CASTING ALLOY

Leslie J. Larrien, San Marino, Calif., assignor to Morris P. Kirk & Son, Inc., Los Angeles, Calif., a corporation of Nevada  
No Drawing. Filed May 4, 1966, Ser. No. 547,407  
U.S. Cl. 75—178 12 Claims  
Int. Cl. C22c 17/00

### ABSTRACT OF THE DISCLOSURE

Improved zinc base die casting alloys conforming to A.S.T.M. specification Alloy XXIII and Alloy XXIII modified with small additions of nickel, both alloys improved in mechanical strength retention after aging by the addition of small but critical amounts of beryllium.

This invention relates to zinc base casting alloys and has for its object the provision of an improved alloy conforming in composition limits generally to A.S.T.M. B86-64, Alloy AG40A, commonly called Alloy XXIII and hereafter referred to as Alloy XXIII. Specifically the invention provides for a small but critical element addition of beryllium to Alloy XXIII and to Alloy XXIII modified with small amounts of nickel, which, when cast, retains substantially more mechanical properties after aging than the same alloys would without the critical element addition.

A.S.T.M. B86-64 Alloy AG40A (XXIII)

|                | Percent   |
|----------------|-----------|
| Copper (max.)  | .25       |
| Aluminum       | 3.5—4.5   |
| Magnesium      | .02—.05   |
| Iron (max.)    | .10       |
| Lead (max.)    | .005      |
| Cadmium (max.) | .004      |
| Tin (max.)     | .003      |
| Zinc           | Remainder |

The A.S.T.M. Alloy XXIII with composition limits as listed above enjoys a very large usage in the manufacture of zinc base castings. This alloy possesses very good fluidity and castability, however, it does possess the objectionable property of losing a substantial part of its good mechanical properties, particularly, the important tensile strength property, after aging over periods of six months to five years at room temperature and after shorter intervals of time when temperatures in excess of room temperature are encountered. The mechanical properties most substantially affected are tensile strength and hardness. Impact strength is relatively unaffected by aging changes.

In like manner the A.S.T.M. Alloy XXIII, when modified by a substitution of a small amount of nickel to compensate for the use of a lower amount of magnesium, is similarly affected by loss of tensile properties after aging period at room temperature. The use of the lesser amount of magnesium is made in order to achieve better castability for the alloy and the addition of nickel to the alloy provides compensatory corrosion protection.

It is well known by those informed about zinc alloy metallurgy that the binary alloy of zinc-aluminum, containing 3.5%—4.5% aluminum and .005%—.05% magnesium is subject to at least one phase change during aging. It is also well known that during that during these changes in phase relationship there occurs a substantial reduction in the amount of mechanical properties when compared to those possessed in the "as cast" state. Mechanical properties, chiefly tensile strength and hardness, and dimensional properties such as shrinkage and expansion are in-

volved. The expected behaviours are a loss in tensile strength and a loss in hardness accompanied by a very slight shrinkage on the order of .006" in 6".

It is also well known that the addition of small amounts of magnesium such as .005%—.05% retards the transformation and contributes both to better "as cast" mechanical properties and to some retention of those properties after aging.

I have discovered that the addition of small amounts of beryllium such as .0005%—.01% to the A.S.T.M. XXIII Alloy containing aluminum 3.5%—4.3%, copper .25% max., magnesium .02%—.05%, iron .10% max., lead .005% max., cadmium .004% max., tin .003% max., balance special high grade zinc, either retards the phase change or strengthens the transformed phase thus producing an alloy with more retained mechanical properties after aging than an identical composition alloy without beryllium.

I have found that about .002% to about .005% is the optimum range for beryllium and that about .01% beryllium is the maximum amount and that a minimum amount of beryllium is about .0005%, and that about .004% is a preferred optimum amount.

Specifically, I have discovered that the range for beryllium is definitely critical in the sense that there is a minimum below which beneficial results of strength retention after aging are not obtained and a maximum above which beneficial results of strength retention after aging are not obtained in proportion to the increased amount of beryllium added.

Table A lists the retention effects of very small beryllium additions to the XXIII Alloy and Table B lists the comparative retention effects of a .005% beryllium and .010% beryllium to the XXIII Alloy.

TABLE A.—THE EFFECTS OF SMALL ADDITIONS OF BERYLLIUM TO XXIII ALLOY

| Lot  | Composition |     |      |       | Tensile strength in p.s.i. |               |
|------|-------------|-----|------|-------|----------------------------|---------------|
|      | Al          | Cu  | Mg   | Be    | As Cast                    | 18 mos. at RT |
| 2875 | 4           | .08 | .032 | 0     | 44,535                     | 41,432        |
| 2877 | 4           | .08 | .033 | .0001 | 43,616                     | 41,636        |
| 2878 | 4           | .08 | .033 | .0002 | 43,045                     | 41,487        |
| 2919 | 4           | .08 | .033 | .0005 | 45,106                     | 42,044        |

TABLE B.—THE EFFECTS OF LARGER ADDITIONS OF BERYLLIUM TO XXIII ALLOY

| Lot  | Composition |     |      |      | Tensile strength in p.s.i. aged at RT |         |         |
|------|-------------|-----|------|------|---------------------------------------|---------|---------|
|      | Al          | Cu  | Mg   | Be   | As cast                               | 2½ yrs. | 5 years |
| 1498 | 4.0         | .07 | .005 | .005 | 43,065                                | 42,861  | 40,412  |
| 1499 | 4.0         | .14 | .005 | .010 | 45,514                                | 44,086  | 40,616  |

The results listed in Table A confirm an indicated minimum addition of beryllium of about .0005%.

The results listed in Table B present a substantial superiority for the .01% beryllium addition for the conditions of "as cast" and "aged 2½ years at room temperature," however, it is apparent that for the longer term five year period, the two beryllium additions of .005% and .01% impart about equivalent retention properties.

Additional consideration of some reduced ductility from larger beryllium additions and the cost of the alloy addition, when compared to the retention obtained, limit the maximum addition to an amount of about .01% beryllium.

I have also discovered that the addition of small amounts of beryllium such as .0005%—.010% to the

A.S.T.M. Alloy XXIII modified with nickel in amounts ranging from about .005% to about .05%, retards and/or strengthens the phase and produces an alloy with more retained mechanical properties after aging than an identical compositioned alloy without beryllium. I can add nickel in the range of about .005% to about .02% with the optimum amount of about .01%. I have found that the same optimum range, minimum amount and maximum amount of beryllium listed for Alloy XXIII are equally applicable to the modified Alloy XXIII.

The specification for Alloy XXIII lists a maximum copper content of .25%. This limit for copper was set in order to insure the preservation of minimum dimensional changes after aging and to eliminate the possibility of reduced ductility also after long term aging. These changes in ductility and dimension after aging for Alloy XXIII remain constant for copper contents up to about .40% copper and it is now felt that copper contents up to this level will not materially change the characteristics of the XXIII alloy. The .25% maximum copper in the specification amply provides for the preservation of these properties.

I have found that copper in the range of .05% to .40% possesses some increased benefit for strength retention but adds more to the retention of hardness after long term room temperature aging.

I have also discovered that even though beryllium alone exerts a substantial amount of retarding or strengthening influence on the transformation of Alloy XXIII during aging, it is the combined effect of magnesium in the range about .005% to about .05% and of beryllium in the range .0005%-.01% that produces the valuable properties of mechanical strength retention after aging. And with regard to the amount of magnesium, I have discovered that intermediate amounts in the range of about .01% to about .03% may be desirable for strength retention with the optimum amount of about .02%.

The following mechanical property listings are presented in tabular form and are typical representations of the revealed discoveries. The examples present mechanical property data for various compositions within the specification tolerance of A.S.T.M. XXIII and include compositions both with and without beryllium. Also included are mechanical property data for various compositions described as a modified XXIII alloy containing small amounts of substitutional nickel for reduced amounts of magnesium.

Tables I, II, III, VII and VIII list tensile strength properties for aging periods of 60 days and two years under normal conditions of room temperature as well as the "as cast" tensile properties which were obtained in all instances 24 hours after casting.

Table IV presents tensile data for an aging period of eight months at room temperature as well as the "as cast" tensile properties. Table V lists the longer term tensile properties after two and a half years and five years aging at room temperature as well as the "as cast" properties. Table VI lists the properties of impact strength and hardness obtained after the long term aging period of five years as well as the "as cast" properties.

TABLE I.—EFFECT OF BERYLLIUM IN THE PRESENCE OF MAGNESIUM AND THE ABSENCE OF COPPER-DIE CAST

| Lot       | Composition |    |     |      | Tensile strength in p.s.i. |               |               |
|-----------|-------------|----|-----|------|----------------------------|---------------|---------------|
|           | Al          | Cu | Mg  | Be   | As cast                    | 60 days at RT | 2 years at RT |
| 3532----- | 4           | 0  | .02 | 0    | 41,024                     | 39,800        | 35,922        |
| 3558----- | 4           | 0  | .02 | .005 | 45,106                     | 42,861        | 39,500        |

It will be noted that the beryllium bearing alloy exhibits a 4082 p.s.i. advantage as cast, a 3061 p.s.i. advantage after aging 60 days at room temperature and a 3578 p.s.i. superiority after aging two years at room temperature.

TABLE II.—EFFECT OF BERYLLIUM IN THE PRESENCE OF MAGNESIUM AND COPPER-DIE CAST

| Lot       | Composition |     |     |      | Tensile strength in p.s.i. |               |               |
|-----------|-------------|-----|-----|------|----------------------------|---------------|---------------|
|           | Al          | Cu  | Mg  | Be   | As cast                    | 60 days at RT | 2 years at RT |
| 3657----- | 4           | .10 | .02 | 0    | 45,310                     | 41,290        | 36,738        |
| 3678----- | 4           | .10 | .02 | .002 | 43,269                     | 41,432        | 38,983        |

It will be noted that the comparison favors the beryllium free alloy in the "as cast" condition, however, the two alloys are substantially equivalent after aging 60 days at room temperature, but after the long term aging period of two years the strength retention properties imparted by the presence of beryllium are quite evident.

TABLE III.—EFFECT OF BERYLLIUM IN THE PRESENCE OF MAGNESIUM AND NICKEL, AND THE ABSENCE OF COPPER-DIE CAST

| Lot       | Composition |    |     |     |      | Tensile strength in p.s.i. |               |               |
|-----------|-------------|----|-----|-----|------|----------------------------|---------------|---------------|
|           | Al          | Cu | Mg  | Ni  | Be   | As cast                    | 60 days at RT | 2 years at RT |
| 3656----- | 4           | 0  | .02 | .02 | 0    | 43,065                     | 41,024        | 36,738        |
| 3659----- | 4           | 0  | .02 | .02 | .005 | 43,473                     | 41,636        | 38,963        |

It is significant that the two alloys are substantially equivalent in strength properties through 60 days at room temperature and that retention superiority is substantial after two years of room temperature aging for the alloy with the .005% beryllium addition.

TABLE IV.—EFFECT OF BERYLLIUM IN THE PRESENCE OF MAGNESIUM AND COPPER, AND BOTH WITH AND WITHOUT NICKEL-DIE CAST

| Lot       | Composition |     |      |      |       | Tensile strength properties |                |  |
|-----------|-------------|-----|------|------|-------|-----------------------------|----------------|--|
|           | Al          | Cu  | Mg   | Ni   | Be    | As cast                     | 8 months at RT |  |
| 3493----- | 4           | .10 | .008 | .03  | 0     | 43,881                      | 39,187         |  |
| 3501----- | 4           | .10 | .008 | .026 | .0018 | 43,065                      | 40,412         |  |
| 3506----- | 4           | .10 | .008 | 0    | .0014 | 44,002                      | 41,228         |  |

It is significant that the nickel alloy with beryllium retains 1255 p.s.i. more tensile strength than the nickel alloy without beryllium after the moderate term aging period of eight months, however, it is even more significant that the beryllium bearing alloy without nickel retains more strength than either the nickel alloy alone or the nickel alloy with beryllium.

The following tensile strength data listed in Table V illustrates the retentive effect of beryllium upon the A.S.T.M. Alloy XXIII containing very small amounts of copper and the effects of magnesium alone at various concentrations upon retention of tensile properties after long term aging periods of two and a half years and five years at room temperature.

TABLE V.—EFFECT OF MAGNESIUM ALONE AND MAGNESIUM WITH BERYLLIUM-DIE CAST

| Lot       | Composition |     |      |      | Tensile strength properties in p.s.i. |               |               |
|-----------|-------------|-----|------|------|---------------------------------------|---------------|---------------|
|           | Al          | Cu  | Mg   | Be   | As cast                               | 2½ yrs. at RT | 5 years at RT |
| 1364----- | 4.0         | .01 | .006 | 0    | 46,432                                | 40,412        | 37,963        |
| 1365----- | 4.0         | .01 | .020 | 0    | 46,432                                | 40,412        | 38,575        |
| 1395----- | 4.0         | .01 | .050 | 0    | 46,126                                | 38,371        | 37,350        |
| 1399----- | 4.0         | .03 | .030 | .001 | 46,167                                | 42,423        | 40,820        |
| 1400----- | 4.0         | .05 | .030 | .005 | 45,514                                | 43,882        | 41,220        |

These mechanical property data further substantiate the improved tensile strength properties imparted to the XXIII Alloy composition with small addition of beryllium. These tensile strength properties also indicate that neither the low amount of .006% magnesium nor the high amount of .05% magnesium is as desirable from the retained strength objective as the .02% magnesium

addition and that .005% beryllium imparts additional strength retention over the .001% beryllium addition.

The following comparative listing, Table VI presents the Charpy impact properties and the Brinell hardness properties for all of the alloy compositions listed in Table V and after the aging periods as designated in that table.

TABLE VI.—EFFECT OF MAGNESIUM ALONE AND MAGNESIUM WITH BERYLLIUM

| Lot       | Composition |     |      |      | Charpy impact |               | Brinell hardness |               |
|-----------|-------------|-----|------|------|---------------|---------------|------------------|---------------|
|           | Al          | Cu  | Mg   | Be   | As cast       | 5 years at RT | As cast          | 5 years at RT |
| 1364----- | 4.0         | .01 | .006 | 0    | 40.0          | 38.5          | 85.7             | 74.1          |
| 1365----- | 4.0         | .01 | .020 | 0    | 39.6          | 39.0          | 89.0             | 76.8          |
| 1398----- | 4.0         | .01 | .050 | 0    | 36.8          | 38.0          | 92.6             | 74.1          |
| 1399----- | 4.0         | .03 | .030 | .001 | 38.0          | 38.5          | 89.0             | 79.6          |
| 1400----- | 4.0         | .05 | .030 | .005 | 38.5          | 40.0          | 92.6             | 82.6          |

It is readily evident that impact strength is neither affected by the compositions and alloy contents listed nor by the aging time and conditions employed. This property remains good for the XXIII Alloy under most conditions of time and exposure.

The Brinell hardness properties parallel the tensile properties to some extent and it is significant to note that the two beryllium bearing alloys, 1399 and 1400, lost about 10 points Brinell each after aging five years whereas the beryllium free alloys lost a greater amount in each instance.

Many large die casting operations employ the practice of quenching the cast parts as they are ejected quite hot from the die casting machine. The usual practice is to use a water soluble oil emulsion solution. This practice constitutes a somewhat severe quench and produces somewhat superior mechanical properties for the parts in the "as cast" condition, particularly Brinell hardness.

Table VII presents the tensile strength properties for the XXIII Alloy containing .10% copper and .02% magnesium and the effect of .005% beryllium on that composition quenched and aged. Table VIII lists similar test results for a comparable XXIII Alloy containing .05% nickel and also quenched.

TABLE VII.—EFFECT OF BERYLLIUM ON XXIII ALLOY WITH .10% COPPER-DIE CAST AND QUENCHED

| Lot       | Composition |     |     |      | Tensile strength properties |               |
|-----------|-------------|-----|-----|------|-----------------------------|---------------|
|           | Al          | Cu  | Mg  | Be   | As cast                     | 2 years at RT |
| 3566----- | 4.0         | .10 | .02 | 0    | 44,902                      | 37,146        |
| 3567----- | 4.0         | .10 | .02 | .005 | 46,331                      | 40,004        |

It is evident that the long term aging at room temperature reduces the "as cast" tensile strengths obtained from quenching down to the levels obtained for similar compositioned unquenched specimens. The superior tensile strength retention properties imparted by the beryllium addition are evident.

TABLE VIII.—EFFECT OF BERYLLIUM ON XXIII ALLOY WITH .10% COPPER AND .05% NICKEL-DIE CAST AND QUENCHED

| Lot       | Composition |     |     |     |      | Tensile strength properties |               |
|-----------|-------------|-----|-----|-----|------|-----------------------------|---------------|
|           | Al          | Cu  | Mg  | Ni  | Be   | As cast                     | 2 years at RT |
| 3599----- | 4           | .10 | .02 | .05 | 0    | 45,106                      | 37,963        |
| 3598----- | 4           | .10 | .02 | .05 | .005 | 46,697                      | 40,208        |

It is evident that the presence of nickel has contributed some additional tensile properties to both the beryllium free alloy and the beryllium bearing alloy, however, it 75

is quite evident that the conditions of quenching and the presence of nickel do not alter the retentive properties imparted by the presence of a small addition of beryllium.

These examples and comparisons demonstrate the effect that beryllium bears upon the tensile strength of Alloy XXIII after moderate to long term periods of aging at room temperature. The observed improvement either results from retarding the rate of change and hence the total amount of change in phase relationships or the small beryllium addition imparts a strengthening effect upon the weaker phase produced by transformation.

Some credence can be placed in the latter hypothesis from the study of many photomicrographs depicting the microstructure of comparative compositions.

The 4% aluminum balance zinc composition is comparatively very coarse. The addition of magnesium to this composition refines the structure and produces a random constituent distribution, whereas the addition of beryllium in the presence of magnesium refines the resultant microstructure and produces a marked improvement in the homogeneity of constituent distribution. Beryllium appears to alter the microstructures by dispersing the constituents that, otherwise in the absence of beryllium, agglomerates into very visible discrete entities at 200 $\times$  magnification.

Thus it has been revealed and demonstrated that the alloy of this invention, conforming in composition to A.S.T.M. B86-64 Alloy XXIII and with additions of beryllium in the range .0005% to .01%, represents an important advance in the art with respect to zinc base die casting alloys and the die cast parts produced with the improved alloy.

It has also been revealed and demonstrated that the alloy of this invention may be modified in composition to the extent that it may contain reduced amounts of magnesium such as .005% with small additions of compensatory nickel such as .01%-.05% and copper slightly in excess of the maximum .25% such as maximum .40% and all such modified compositions with beryllium in the range .0005%-.01%.

This discovery alloy can be of great benefit to the zinc alloy die casting industry and to the related industries served. The availability of this discovery alloy will enable design engineers to incorporate zinc alloy die castings into machine assemblies with confidence that the limiting factor of life expectancy for the designed machine assembly will not be the failure of the XXIII Alloy die cast parts caused by substantial loss of tensile strength after aging periods of one to five years or longer.

Tensile strength is the most significant and determinative property for cast parts to possess and every pound per square inch that can be retained during service use is of critical importance for the extension of the life of the die cast part and the machine assembly of which it is a part.

The alloy of this invention may be produced by any of the accepted methods familiar to those skilled in the art. The beryllium addition can be made either from the commercial aluminum-beryllium alloy containing approximately 5% beryllium or from a copper-aluminum-beryllium master alloy manufactured by melting a sufficient amount of pure aluminum (25 lbs.) in a #40 or #30 graphite crucible at about 1500° F. after which a predetermined amount (30 lbs.) of 96% copper-4% beryllium alloy is added. This produces 55 lbs. of master alloy of the following composition: copper 52.3%, aluminum 45.3% and beryllium 2.37%.

The following kinds and quantities of raw materials will produce one ton of the alloy of the invention:

|                                   | Pounds |
|-----------------------------------|--------|
| Zinc (special high grade 99.99+%) | 1920.0 |
| Aluminum (E.C. grade 99.8%)       | 78.5   |
| Magnesium (pure stick)            | .4     |
| Beryllium (Cu-Al-Be master)       | 4.0    |

A specific manufacturing procedure calls for the addition of 78.5 lbs. of pure aluminum to 1920 lbs. of pure zinc at 900° F. After the aluminum is all in solution and with the temperature at 900° F. add 4 lbs. of the Cu-Al-Be master. This master alloy is added in small walnut sized pieces and solution is helped by gentle agitation. After the master alloy is in solution the pot is stirred, skimmed and the magnesium is added. After another stirring and skimming the pot is ready to cast.

The resultant composition will be: aluminum 4.0%, copper .10%, magnesium .02%, beryllium .004%, and the remainder zinc, with combined lead, cadmium and tin less than .012%.

If a nickel content is desired in order to produce the modified XXIII Alloy of the invention with nickel, a zinc-nickel master alloy addition or an aluminum-nickel master alloy addition can be made at the time of the aluminum addition to the zinc.

If a copper free XXIII Alloy of the invention is desired, add sufficient aluminum-beryllium master to introduce the desired amount of beryllium.

I claim:

1. A zinc base die cast alloy of high purity containing beryllium additions for imparting retention of tensile strength properties after being subjected to prolonged aging, consisting by weight essentially of about 3.0% to about 5.0% aluminum, about .02% to about .05% magnesium, about .0005% to about .005% beryllium and the remainder zinc with iron not in excess of .10% and the combined impurities of lead, cadmium and tin not present in excess of .012% total.

2. A zinc base die cast alloy of high purity containing beryllium additions for imparting retention of tensile strength properties after being subjected to prolonged aging, consisting by weight essentially of about 3.0% to about 5.0% aluminum, about .005% to about .40% copper, about .02% to about .05% magnesium, about .0005% to about .005% beryllium and the remainder zinc with iron not present in excess of .10% and lead not present in excess of .005%, cadmium not present in excess of .004% and tin not present in excess of .003%.

3. A zinc base die cast alloy of high purity containing beryllium additions for imparting retention of tensile strength properties after being subjected to prolonged aging, consisting by weight essentially of about 3.0% to about 5.0% aluminum, about .005% to about .40% copper, about .005% to about .05% magnesium, about .005% to about .05% nickel, about .0005% to about .01% beryllium and the remainder zinc with iron not in excess of .10% and the combined impurities of lead, cadmium and tin not present in excess of .012% total.

4. A zinc base die cast alloy of high purity containing beryllium additions for imparting retention of tensile strength properties after being subjected to prolonged aging, consisting by weight essentially of about 3.0% to about 5.0% aluminum, about .005% to about .05% magnesium, about .005% to about .05% nickel, about .0005% to about .01% beryllium and the remainder zinc with iron not in excess of .10% and the combined impurities of lead, cadmium and tin not present in excess of .012% total.

5. A zinc base die cast alloy of high purity containing beryllium additions for imparting retention of tensile strength properties after being subjected to prolonged aging consisting essentially of the following by weight:

|               |           |
|---------------|-----------|
| Aluminum      | 3.5-4.5   |
| Magnesium     | .005-.03  |
| Beryllium     | .001-.005 |
| Iron, max.    | .10       |
| Lead, max.    | .005      |
| Cadmium, max. | .004      |
| Tin, max.     | .003      |
| Zinc          | Remainder |

6. A zinc base die cast alloy of high purity containing beryllium additions for imparting retention of tensile strength properties after being subjected to prolonged aging consisting essentially of the following by weight:

|    |               |           |
|----|---------------|-----------|
| 5  | Aluminum      | 3.5-4.5   |
|    | Copper        | .005-.25  |
|    | Magnesium     | .005-.03  |
|    | Beryllium     | .001-.005 |
|    | Iron, max.    | .10       |
| 10 | Lead, max.    | .005      |
|    | Cadmium, max. | .004      |
|    | Tin, max.     | .003      |
|    | Zinc          | Remainder |

7. A zinc base die cast alloy of high purity containing beryllium additions for imparting retention of tensile strength properties after being subjected to prolonged aging consisting of the following by weight:

|    |               |           |
|----|---------------|-----------|
| 15 | Aluminum      | 3.5-4.5   |
|    | Copper        | .005-.25  |
|    | Magnesium     | .005-.03  |
|    | Nickel        | .005-.02  |
|    | Beryllium     | .001-.005 |
|    | Iron, max.    | .10       |
| 20 | Lead, max.    | .005      |
|    | Cadmium, max. | .004      |
|    | Tin, max.     | .003      |
|    | Zinc          | Remainder |

8. A zinc base die cast alloy of high purity containing beryllium additions for imparting retention of tensile strength properties after being subjected to prolonged aging consisting essentially of the following by weight:

|    |               |           |
|----|---------------|-----------|
| 25 | Aluminum      | 3.5-4.5   |
|    | Magnesium     | .005-.03  |
|    | Nickel        | .005-.02  |
|    | Beryllium     | .001-.005 |
|    | Iron, max.    | .10       |
| 30 | Lead, max.    | .005      |
|    | Cadmium, max. | .004      |
|    | Tin, max.     | .003      |
|    | Zinc          | Remainder |

9. A zinc base die cast alloy of high purity containing beryllium additions for imparting retention of tensile strength properties after being subjected to prolonged aging consisting essentially by weight of about 3.0% to 5.0% aluminum, about .02% magnesium, about .004% beryllium and the remainder zinc with iron not in excess of .10% and the combined impurities of lead, cadmium and tin not present in excess of .012% total.

10. A zinc base die cast alloy of high purity containing beryllium additions for imparting retention of tensile strength properties after being subjected to prolonged aging consisting essentially by weight of about 3.0% to 5.0% aluminum, about .10% copper, about .02% magnesium, about .004% beryllium and the remainder zinc with iron not in excess of .10% and the combined impurities of lead, cadmium and tin not present in excess of .012% total.

11. A zinc base die cast alloy of high purity containing beryllium additions for imparting retention of tensile strength properties after being subjected to prolonged aging consisting essentially by weight of about 3.0% to about 5.0% aluminum, about .10% copper, about .01% magnesium, about .01% nickel, about .004% beryllium and the remainder zinc with iron not in excess of .10% and the combined impurities of lead, cadmium and tin not present in excess of .012% total.

12. A zinc base die cast alloy of high purity containing beryllium additions for imparting retention of tensile strength properties after being subjected to prolonged aging consisting essentially by weight of about 3.0% to about 5.0% aluminum, about .01% magnesium, about .01% nickel, about .004% beryllium and the remainder

zinc with iron not in excess of .10% and the combined impurities of lead, cadmium and tin not present in excess of .012% total.

## References Cited

## UNITED STATES PATENTS

5

|           |        |         |       |        |
|-----------|--------|---------|-------|--------|
| 2,467,956 | 4/1949 | Bierman | ----- | 75—178 |
| 3,037,859 | 6/1952 | Larrieu | ----- | 75—178 |
| 3,083,096 | 3/1963 | Larrieu | ----- | 75—178 |
| 3,234,016 | 2/1966 | Larrieu | ----- | 75—178 |

## FOREIGN PATENTS

|           |         |                |
|-----------|---------|----------------|
| 1,248,301 | 10/1960 | France.        |
| 1,321,677 | 2/1963  | France.        |
| 913,576   | 12/1962 | Great Britain. |

CHARLES N. LOVELL, *Primary Examiner.*

U.S. Cl. X.R.